

## UNITED STATES PATENT OFFICE

2,008,733

## TREATMENT OF COATINGS

Martin Tosterud, Arnold, Pa., assignor to Aluminum Company of America, Pittsburgh, Pa., a corporation of Pennsylvania

No Drawing. Application May 26, 1932, Serial No. 613,793

## 20 Claims. (Cl. 148—6)

The invention relates to methods of treating oxide coatings, composed in substantial part of aluminum oxide, to alter or modify the properties and characteristics of the coatings. Particularly 5 is the invention concerned with the treatment of oxide coatings formed on aluminum and aluminum base alloy surfaces, herein collectively referred to as aluminum surfaces.

By several known processes aluminum surfaces 10 may be provided with what is generally termed an oxide coating. This coating is substantially composed of aluminum oxide. It may contain, because of the process used, other components which essentially alter its specific characteristics. 15 Such oxide coatings have, as general properties, a good resistance to corrosion, a good resistance to abrasion, and an ability, in various degrees, to take organic dyes or inorganic colors to form a colored surface. The oxide coatings may be 20 more or less permeable and adsorb or absorb moisture or liquids. Quite often, also, the coating forms an excellent insulation against the passage of electric current.

The oxide coatings may be formed on aluminum surfaces by various methods. The aluminum may be made an anode in an electrolytic cell containing an electrolyte such as sulfuric acid, chromic acid, organic acids, acid salts, etc. When external electrical energy is impressed upon 25 the cell an oxide coating is formed on this anode. In another method the aluminum is immersed in a suitable solution, generally alkaline, and the oxide coating is formed by chemical reaction without the use of external electrical energy. 30 Other processes are known and used to produce artificially these oxide coatings. In all cases the oxide coating to which this invention relates is produced by artificial means. The natural film of oxide occurring on all aluminum surfaces is 35 40 not herein referred to as an oxide coating.

The oxide-coated aluminum surface may then be immersed in organic dyes, or in solutions of dyes, to produce characteristic colors.

The object of the present invention is to treat 45 oxide coatings formed on aluminum surfaces to produce certain results, among which may be numbered: a decrease in the permeability of the oxide coating; a modification of the adsorptive 50 or absorptive capacity of the oxide coating for coloring agents; increase in corrosion resistance of the coating; increase of the ability of the colored oxide coating to retain color under the action of solvents. Another object of the invention 55 is to treat colored oxide coatings after the

coloring operation to uniformly fix said color in and on the coating.

The objects are obtained in lesser or greater degree depending upon the particular coating treated and the manner in which the treatments hereinafter described are used, but in every case a new or improved result is obtained which greatly enhances the usefulness of the oxide-coated aluminum and the breadth of its commercial application.

The invention is predicated upon the discovery that by the treatment of oxide-coated aluminum in hot or boiling solutions of certain salts the properties of the coating are considerably modified and new and advantageous properties are 10 developed. The solutions to which this invention refers are solutions containing a salt of a weak metallic base which salt is capable of hydrolyzing in solution to form a substantially insoluble compound of the metal in the oxide coating. 15 The hydrogen ion concentration of the solution should be such that the hydrolysis in hot or boiling solution promotes precipitation of the metal compound and this condition is usually evidenced by the appearance of turbidity in 20 the solution. Among the salts which will form such solutions (with proper hydrogen ion adjustment) are metallic acetates, such as nickel, cobalt, cadmium, zinc, barium, copper, aluminum or lead acetates, and metallic sulfates, oxalates, 25 chlorides, nitrates, citrates, tartrates and fluorides, but there are other salts of similar chemical characteristics which will produce the desired results.

While the invention broadly contemplates the 35 use of such solutions, in its specific and preferred practice certain salts are preferable to others. For instance, because of the difficulty involved in maintaining proper hydrogen ion concentration, solutions of the salts of weak acids and 40 weak metallic bases are preferable in commercial operation, provided that they have the properties of the general class above stated, i. e., especially the property of hydrolyzing in hot or boiling solutions to form a precipitate in the 45 oxide coating. Likewise in specific applications of the practice of the invention, it is often highly desirable that the salt solution be one which does not color the coating and/or it be one which does not leave in the coating a poisonous or toxic element. Also it is desirable from many commercial viewpoints that the salt solution be one that does not materially attack or dissolve the oxide coating or the aluminum. Such preferred properties of 50 the salt solution are, however, desirable only in 55

certain applications of the invention, and the broad class of salt solutions herein defined are, per se, commercially useful.

The solutions used in the practice of the invention are prepared by dissolving a salt of the class described in water and then, if necessary, adjusting the hydrogen ion concentration to the point where hydrolysis in hot or boiling solutions, i. e., in solutions heated above 40° centigrade, will 5 promote precipitation in the oxide coating. The hydrolysis, under these conditions, may be such that suspension of colloidal dimensions is formed in the solution and no precipitate is evident. But if, on heating, a precipitate is evident, the hydrogen ion concentration is so adjusted that a substantial amount of the metallic base is not precipitated in flocculent form and does not settle from the solution. In solutions where, on hydrolysis, precipitation is evident, it is desirable that the 10 hydrolysis does not substantially proceed past the point of turbidity. The term "turbidity" as used herein and in the appended claims denotes not only a turbid but likewise an opalescent or cloudy solution. In the practice of my invention 15 with preferred solutions such turbidity is customarily observed. The proper hydrogen ion concentration is readily predetermined by simple experiment, but it is preferred and usually advisable to use solutions having a hydrogen ion concentration, as measured at 25° centigrade, of between a pH of about 4.5 and a pH of about 7.5. When the solution has pH values widely variant 20 from this range, the proper solution conditions are not usually obtained and, moreover, the oxide-coated aluminum will be attacked. In the case of each solution, however, the proper hydrogen ion concentration is readily and simply determined by experiment, such as by immersing several pieces of oxide-coated aluminum in solutions 25 of varying hydrogen ion concentration and observing the results obtained thereby.

When the salt is one of a weak metallic base and a strong acid it is very desirable to add to the solution a buffer such as boric acid, borates, 30 acetates, or other well known buffering agents, in order that the proper hydrogen ion concentration may be readily obtained and maintained, the buffering agent tending to reduce the sensitivity of the adjustment. Likewise when, in 35 preferred practice, a salt of a weak base and a weak acid is used, the employment of a buffering agent may be desirable in the interests of maintaining the predetermined hydrogen ion concentration desired. For instance, excellent results 40 have been obtained by adding boric acid to solutions of nickel or cobalt acetate.

The salt solution may contain large or small amounts of a salt of the general class described. While amounts of 0.1 per cent by weight have 45 been found efficient, and solutions containing the salt to the maximum solubility thereof are useful, it is preferable in commercial solutions, when solubility relations permit, to use about 1 or 2 per cent of the salt in solution. From time to 50 time the solution may have to be renewed as it becomes exhausted or inactive by use.

The oxide-coated aluminum is immersed in the hot or boiling salt solution for a time sufficient 55 to effect the result desired. The time of treatment varies with the particular coating and with the particular effect desired. It is usually between about 2 and 30 minutes.

In order to describe the effects obtained, several of the uses to which the methods of the

invention may be placed will be specifically mentioned.

Quite often the oxide coating is placed upon aluminum utensils such as trays, ice-freezing receptacles and the like. In such cases the coating is not colored since the natural oxide-coated aluminum finish is desired. Such trays and receptacles are often in contact with colored liquids, colloidal or otherwise, and such liquids, if adsorbed by the oxide coating, stain the coating. By treating the coated articles in salt solutions in accordance with this invention, the coating is made substantially non-porous and impermeable, thus eliminating or materially decreasing the propensity of the coating to stain. When 10 the methods of the invention are thus used, it is desirable to employ salt solutions which do not, themselves, color the oxide coating or act as a mordant for coloring agents.

Or, again, the aluminum article may have 20 been provided with a colored oxide coating or with a coating containing in its pores a substance such as sodium silicate, which will increase the corrosion resistance of the coating. Such a coated aluminum article may, in its use, be subject to detrimental external agencies such as moisture, general weather conditions, solvents, etc., which will tend to remove the coloring or other materials from the pores of the coating. By treating the coated article in accordance with 25 this invention, in salt solutions of the class described, the coating is made impermeable or substantially so; and, at the same time, the useful substance, coloring matter or otherwise, is more or less permanently bound in the pores 30 of the oxide coating and protected against the action of solvents, etc.

When an oxide-coated aluminum article is dipped into a solution of organic dye, as is commercial practice, most of the dye which remains 40 on the article, after removal from the dye solution and rinsing, is adsorbed in the oxide coating, but a certain amount of the dye lying on or adjacent the coating surface is not so firmly bound to the coating. Consequently this dye 45 tends to rub off in use. To cure this it has been the practice to buff the colored coating, but buffing is often expensive and, in the case of small articles, such as buttons and pins, practically impracticable. By treating the article according to methods of the present invention, the dye on or adjacent the surface is substantially fixed 50 on said surface so that "crocking" or smudging are minimized.

While any of the general class of salt solutions 55 herein defined will give the results described in greater or less degree, there are, as has herein been stated, certain salts which are preferred to others. Among such salts are found those which are used in the preferred commercial practice of 60 my invention; viz., nickel acetate, cobalt acetate, nickel sulfate and cobalt sulfate; of these named salts the acetates are generally preferred. Buffering agents are useful in solutions of either the sulfate or the acetate.

I claim:

1. The method of depositing in an oxide-coated aluminum surface an insoluble compound by hydrolyzing a salt of a weak metallic base in solution, and immersing said oxide-coated aluminum in said solution.

2. The method of depositing in an oxide-coated aluminum surface an insoluble compound formed by hydrolysis of a salt of a weak metallic base, by immersing said oxide-coated aluminum 75

in a solution of a salt of said weak metallic base, and maintaining the temperature of said solution above about 40° centigrade.

3. The method of depositing in an oxide-coated aluminum surface an insoluble compound formed by hydrolysis of a salt of a weak metallic base, by immersing said oxide-coated aluminum in a solution of a salt of said weak metallic base having a pH of 4.5 to 7.5.

10 4. The method of depositing in an oxide-coated aluminum surface an insoluble compound formed by hydrolysis of a salt of a weak metallic base, by immersing said oxide-coated aluminum in a solution of a salt of said weak metallic base having a pH of 4.5 to 7.5, and maintaining the temperature of said solution above about 40° centigrade.

5 5. The method of depositing in an oxide-coated aluminum surface an insoluble compound formed by hydrolysis of a salt of a weak metallic base, by immersing the said oxide-coated aluminum in a solution of a salt of the weak metallic base and a weak acid and maintaining the temperature of the solution above about 40° centigrade.

10 6. The method of treating oxide-coated aluminum surfaces by immersing the same in a solution of a salt of a weak metallic base in which hydrolysis proceeds to the point of turbidity and which contains no substantial amount of flocculent precipitate.

15 7. The method of treating oxide-coated aluminum surfaces by immersing the same in a solution of a salt of a weak metallic base and a weak acid in which hydrolysis proceeds to the point of turbidity and which contains no substantial amount of flocculent precipitate.

20 8. The method of depositing in an oxide-coated aluminum surface an insoluble compound formed by hydrolysis of a salt of a weak metallic base, by immersing said oxide-coated aluminum in a solution of a salt of a weak metallic base which contains also a buffering agent, and maintaining the temperature of said solution above about 40° centigrade.

25 9. The method of depositing in an oxide-coated aluminum surface an insoluble compound formed by hydrolysis of a salt of a weak metallic base, by immersing said oxide-coated aluminum in a solution of a salt of a weak metallic base and a strong acid which contains also a buffering agent, and maintaining the temperature of said solution above about 40° centigrade.

10. The method of depositing in an oxide-coated aluminum surface an insoluble compound formed by hydrolysis of a nickel salt, by immersing said oxide-coated aluminum in a solution of said nickel salt having a pH of 4.5 to 7.5.

10 11. The method of depositing in an oxide-coated aluminum surface an insoluble compound formed by hydrolysis of a cobalt salt, by immersing said oxide-coated aluminum in a solution of said cobalt salt having a pH of 4.5 to 7.5.

15 12. The method of treating oxide-coated aluminum surfaces by immersing the same in a solution of a nickel acetate; the temperature of the solution being above 40° centigrade.

15 13. The method of treating oxide-coated aluminum surfaces by immersing the same in a solution of a nickel acetate; the solution containing also a buffering agent and having a temperature above 40° centigrade.

20 14. The method of treating oxide-coated aluminum surfaces by immersing the same in a solution of nickel sulfate; the temperature of the solution being above 40° centigrade.

25 15. The method of treating oxide-coated aluminum surfaces by immersing the same in a solution of nickel sulfate; the solution containing also a buffering agent and having a temperature above 40° centigrade.

30 16. The method of treating oxide-coated aluminum surfaces by immersing the same in a solution of cobalt acetate; the temperature of the solution being above 40° centigrade.

35 17. The method of treating oxide-coated aluminum surfaces by immersing the same in a solution of cobalt acetate; the solution containing also a buffering agent and having a temperature above 40° centigrade.

40 18. The method of treating oxide-coated aluminum surfaces by immersing the same in a solution of cobalt sulfate; the temperature of the solution being above 40° centigrade.

45 19. The method of treating oxide-coated aluminum surfaces by immersing the same in a solution of cobalt sulfate; the solution containing also a buffering agent and having a temperature above 40° centigrade.

50 20. The method of treating oxide-coated aluminum surfaces by immersing the same in a solution of cobalt sulfate; the solution containing also a buffering agent.

MARTIN TOSTERUD.